

Sept. 5, 1961

D. M. YENNI ET AL

2,998,632

PROCESS OF MAKING SPARK PLUG ELECTRODE STRUCTURES

Filed June 10, 1959

*Fig. 1.*



*Fig. 2.*



*Fig. 3.*



*Fig. 4.*



INVENTORS  
DONALD M. YENNI  
WALTER A. RUNCK

BY *Barnwell P. King*  
ATTORNEY

1

2,998,632

**PROCESS OF MAKING SPARK PLUG ELECTRODE STRUCTURES**

Donald M. Yenni, Indianapolis, Ind., and Walter A. Runck, New York, N.Y., assignors to Union Carbide Corporation, a corporation of New York

Filed June 10, 1959, Ser. No. 819,293

3 Claims. (Cl. 29—25.12)

This invention relates to spark plugs having concentric ring electrodes for internal combustion engines, and more particularly to the manufacture thereof.

The invention provides a novel method of making a unitary electrode structure for spark plugs in which concentric rings of electrode material and insulation are formed at the end of such structure by first spraying onto a suitable base member alternating coating layers of conductive refractory metal, such as tungsten or molybdenum, and refractory insulating material, such as aluminum oxide, by means of an electric arc torch coating process; and then grinding away a portion of such coatings to leave spaced annular electrodes of such conductive metal on the end of the resulting structure.

A recent modification of spark plug apparatus which has been found to be useful for automotive engines comprises two ring-shaped electrodes separated by an annular insulator. Such type of electrode configuration is more resistant to fouling than are the more conventional spark plug electrodes. It is desired that such electrodes be fabricated from high temperature metallic materials, but the industry has been plagued with considerable failure in satisfactorily forming such electrode apparatus.

The main object of this invention is to provide a method of manufacturing spark plug electrode structures, which overcomes such problem of the prior art.

In the drawings:

FIG. 1 is a vertical cross section of a suitable base member.

FIG. 2 is a cross section of a 3-layer coating combination applied to such base member;

FIG. 3 is a cross section of the finished spark plug electrode combination of FIGS. 1 and 2;

FIG. 4 is a vertical cross section of an alternate type of suitable base member having a central passage;

FIG. 5 is a cross section of a finished spark plug using a 3-layer coating combination applied to such base.

A desired electrode configuration can be obtained by using a suitable base 10 of a type similar to that shown in FIG. 1. This base member is preferably of metal but could be of ceramic if desired. A coating 11 of refractory, electrically conductive metal, especially tungsten, is then applied to the end region of the base 10 by means of an electric arc torch plating process. The process using a collimated electric arc as described in patent application Serial No. 706,099, filed on December 30, 1957, is especially useful in this invention. Additional layers of refractory insulating material 12 and refractory electrically conductive metal 13 are then applied to the coated base member in a similar fashion.

In a final step, the coatings are ground off to the point where a desired exposed surface results and where a controlled annular insulator layer 12 is obtained between ring-shaped metal sections 11 and 13. In operation, metal ring 13 is then connected to one terminal of the power supply (not shown) and ring 11 can be connected to the other terminal of the power supply through metal base member 10. If the base member 10 is ceramic, a wire conductor for ring 11 might be embedded in the ceramic base member.

2

It has been found desirable that metal coatings 11 and 13 have a thickness of about 0.010—0.020 inch and that the insulator layer 12 be about 0.010—0.020 inch wide. The insulator layer is preferably 0.010—0.015 inch wide. It is understood that the metal coatings could also contain minor amounts of emissive materials such as yttria or thoria.

This process is described in more detail in the following example.

**EXAMPLE***Multiple layer spark plug*

An arc of 200 amperes and 50 volts was established between a  $\frac{1}{8}$  inch diameter thoriated tungsten cathode 15 and a  $\frac{3}{64}$  inch diameter water-cooled copper nozzle anode while 300 c.f.h. argon passed around the cathode and out through the anode nozzle passage. Tungsten powder (6.8 micron diameter) was passed through the nozzle passage at 31 grams per minute and impinged on the end portion of a steel rod of the type shown in FIG. 1 by means of the high temperature, high velocity gas effluent to form a tungsten coating about 0.015 inch thick. The coating particles impinged onto the base at 20 an angle of about 90°. The tungsten powder flow was then substituted by an alumina powder flow of 11 grams per minute to form a 0.015 inch thick coating of alumina on top of the tungsten. A third 0.015 inch thick coating of tungsten was then applied on top of the alumina. 25 The end portion of the resulting coated body was then ground down to level off the coatings and form the ring-shaped tungsten areas separated by an alumina layer.

It should be noted that the most successful coating results are attained when the coating apparatus and the body being coated are so positioned that the coating particles impinge on the desired surface at an angle of about 90°. Severe angle deviations from this position greatly reduce the quality and bonding strength of the coating.

40 It is also necessary to apply these coatings in a series of short coating intervals of about 3—10 seconds in order to prevent serious over-heating of the relatively small base structures. In a production line setup the spark plugs would probably pass through several coating stations in order to achieve the desired coated body structure.

45 Electrode configurations obtained in the above manner were tested by connecting a magneto across the concentric tungsten electrodes. The magneto was driven by a 1725 r.p.m. motor, and the sparking action in air was observed by means of a microscope. This coated spark plug device was operated under continuous sparking action for several hours with no apparent wear. Additional tests of similar electrodes were made in an internal combustion engine. Simulated operation of thousands of miles of service was obtained without noticeable electrode wear.

50 The specific design of the base material can vary considerably depending on the desired final spark plug configuration, without departing from our invention.

60 As an example of an alternative design, the base member shown in FIG. 4 might be used. For purposes of illustration the use of a metal base will be assumed to aid in cooling the electrodes. Base member 14 could rotate while refractory metal coating 16 and insulation layer 17 are applied. The central portion of the coatings would then be trimmed or ground to form an extension of passage 15 in base member 14. An electrical conductor 18 could then be passed through passage 15. Final refractory metal coating 19 could then be applied to the insulation layer and to the end of conductor 18 while rotating the base member. The outer edges of

the three layers would then be ground to the finished dimension. FIG. 5 shows a cross section of the finished electrode structure. Electrical connection to electrode 16 could be made through an outer conductor (not shown).

What is claimed is:

1. Process of making spark plugs having concentric ring electrodes for internal combustion engines, which comprises the steps of electric arc spraying consecutive layers of refractory electrode metal, refractory insulating material and refractory electrode metal onto the end region of a suitable base member, and grinding away an end portion of the coatings to provide spaced annular electrode surfaces on the end region of the base member.

2. Process of making spark plugs having concentric ring electrodes for internal combustion engines, which comprises the steps of electric arc spraying 0.010-0.020 inch thick consecutive layers of refractory electrode

metal, refractory insulating material and refractory electrode metal onto the end region of a suitable base member, and grinding away an end portion of the coatings to provide spaced annular electrode surfaces on the end region of the base member.

5 3. Process of making spark plugs having concentric ring electrodes for internal combustion engines, which comprises the steps of electric arc spraying consecutive coatings of tungsten, alumina and tungsten on the end 10 region of a steel base member, and grinding away an end portion of such coatings to provide on such end region of the steel base concentric tungsten electrode rings separated by an insulating alumina ring.

15 References Cited in the file of this patent

UNITED STATES PATENTS

2,265,352 Corbin et al. ----- Dec. 9, 1941  
2,864,152 Peras ----- Dec. 16, 1958